

1

2,711,960

TITANIUM BASE ALLOYS WITH ALUMINUM,  
MANGANESE, AND CHROMIUM

Paul S. Methe, Cohes, N. Y., assignor to Allegheny Ludlum Steel Corporation, Brackenridge, Pa., a corporation of Pennsylvania

No Drawing. Application November 17, 1953,  
Serial No. 392,749

3 Claims. (Cl. 75—177)

This invention relates to titanium-base alloys, and in particular to titanium-base alloys containing aluminum and beta stabilizers.

Heretofore titanium-base binary alloys containing aluminum in excess of 6% have been prepared in limited quantity since considerable difficulty has been experienced in their fabrication. The most notable difficulty experienced thus far has been edge cracking during cold working operations. These difficulties have been attributed to inherent toughness and low ductility of the binary titanium-aluminum alloys. What little ductility these alloys possess is substantially reduced when the binary titanium-aluminum alloys are heated to a temperature in excess of 1700° F., either for the purpose of fabrication or heat treatment.

Since aluminum has the effect of raising the alpha to alpha plus beta transus temperature, the alloy system of aluminum and titanium would appear to be quite desirable from the standpoint of elevated temperature service, especially in the range from 800° F. to 1200° F. However, while the binary alloys of the titanium-aluminum system have the requisite high temperature stability, they do not possess sufficient ductility when the aluminum content is greater than 6% to permit them to be commercially fabricated.

An object of this invention is to provide a titanium-base alloy having a relatively high aluminum content and having small but critical amounts of manganese and chromium.

Another object of this invention is to provide a titanium-base alloy having a substantial amount of aluminum and small but critical percentages of manganese and chromium, the alloy being characterized by retaining substantial ductility after being heated to a temperature of 1700° F.

A further object of this invention is to provide a titanium-base alloy having aluminum, manganese and chromium contained therein, the alloy having a structure consisting of the beta phase in a matrix of the alpha phase with the alpha phase being predominant, said alloy having good ductility after having been forged at a temperature in the range between 1700° F. and 2000° F.

Another object of this invention is to provide a titanium-base alloy having aluminum and small but critical amounts of manganese and chromium contained therein, the alloy being characterized by having excellent elevated temperature creep-rupture properties.

These and other objects of this invention will become apparent to those skilled in the art when read in conjunction with the following description.

In accordance with this invention the titanium alloys of this invention are composed of aluminum in the range from 6.5% to 10%, and small but critical amounts of two beta stabilizers consisting of manganese and chromium. Each of the beta stabilizers present in the alloy is preferably maintained within the range between 0.75% and 1.25%. The balance of these alloys is composed of titanium with incidental impurities, such as not more than

2

0.20% oxygen, not more than 0.15% nitrogen, and not more than 0.10% carbon. In all cases the impurities are preferably maintained at a minimum. Reference is made to the alloys of this invention as set forth in Table I, illustrating the general range, the optimum range, and a specific alloy identified as K-1025.

Table I

| Element | General Range | Optimum Range | K-1025 |
|---------|---------------|---------------|--------|
| Al      | 6.5-10        | 7-9           | 7.00   |
| Mn      | 0.75-1.25     | 0.85-1.15     | 1.00   |
| Cr      | 0.75-1.25     | 0.85-1.15     | 1.14   |

In all cases the balance of the alloys of Table I is titanium with incidental impurities.

The alloys of this invention can be prepared in any well-known manner, for example, by tungsten arc melting, or the consumable arc melting processes. In order to introduce a specific amount of the alloying elements into the titanium base and thereby obtain the titanium-base alloy of the desired chemical composition, the alloying additions may be made in the form of either virgin metals, aluminum master alloy, or a combination of both. However, the manner of addition will depend upon the type of melting employed, namely, tungsten arc melting, or consumable arc melting. When the tungsten arc melting is employed, the alloying elements are blended with the titanium sponge, and the blended mixture is introduced into the molten pool of metal which is formed by the passage of electrical energy between the tungsten electrode and the metal charge, thus creating an arc and thereby melting the metal. On the other hand, if a consumable electrode is employed in arc melting the alloys, the alloying components are preferably added as part of the consumable electrode per se.

Since aluminum has the effect of raising the alpha to alpha plus beta transus temperature and the alpha plus beta to beta transus temperature in a titanium-base alloy, the temperature range under which the alpha phase exists is much broader where the aluminum is a component of the alloy. However, since the alpha phase has a "close-packed hexagonal" crystallographic lattice configuration, it exhibits low ductility in comparison to the "body-centered cubic" structure of the beta phase. To overcome the low ductility of the "close-packed hexagonal" lattice structure of the alpha phase, small but critical amounts of beta stabilizers, which form a "body-centered cubic" crystallographic lattice of the beta phase and which exhibits considerable ductility, are added to the titanium-aluminum-base alloy to increase the over-all ductility of these alloys. At the same time, however, the beta stabilizers do not prove detrimental to the creep-rupture properties nor the alpha stability at elevated temperatures. In so doing, the toughness exhibited by the alpha phase will remain, but the alloys will have sufficient ductility to be fabricated economically.

It has been found also that small but critical percentages of each beta stabilizer has a more desired effect than larger percentages of either one. For example, it has been found that the effect of about 1% manganese and about 1% chromium has a greater beneficial effect for the purposes of these alloys than about 2% of either manganese or chromium. While the reason for accomplishing this effect is not clear, it is believed that each element has a multiplying effect on the over-all alloy rather than an additive effect.

In order to fabricate the alloys of this invention, such as the alloy identified as K-1025 in Table I, it may be forged from a temperature in the range between 1750° F. and 2000° F. The step of forging is performed on the

cast ingot to break up the "as-cast" structure. After forging, the ingot may be rolled in a conventional manner, as will hereinabove be described. The forged alloys are preferably preheated to a temperature of 1400° F. where they are held for a period of about two (2) hours, or until such time as the ingot has soaked to a uniform temperature of 1400° F. Of course, as is well-known, the time to soak to a uniform temperature will vary with the bulk of the metal employed. After the ingot has attained a uniform temperature of 1400° F., the temperature is raised to 1650° F. where it is held for a period of about one half hour to develop a substantially uniform temperature, and thereafter the forged alloy is hot rolled to the desired size in any conventional rolling mill.

As an example of the heating and rolling procedure employed in the fabrication of the alloys of this invention, alloy K-1025, hereinbefore referred to, was processed in the following manner. This alloy, an eleven-pound ingot, was forged at a temperature of 1850° F. to a 2.55" x 2.25" billet, after which it was allowed to cool in air. The billet was then preheated to 1450° F. for two (2) hours, after which time it was heated to 1650° F., held at this temperature for about one half hour, and thereafter hot rolled to a  $\frac{5}{8}$ -inch round bar. Reference may be had to the alloys K-1025 and K-803 in Table II for the purpose of comparing the room temperature tensile properties. Alloy K-1025 was referred to in Table I, while alloy K-803 is a binary titanium-aluminum alloy containing 8% aluminum.

Table II

| Alloy  | Heat Treatment (air cooled)                | T. S.,<br>p. s. i. | T. Y. S.,<br>p. s. i. | El.,<br>percent | R. A.,<br>percent | Re   |
|--------|--------------------------------------------|--------------------|-----------------------|-----------------|-------------------|------|
| K-1025 | As rolled                                  | 192,500            | 190,500               | 16.0            | 31.4              | 44.0 |
|        | 1 hr. @ 1,700° F.                          | 154,500            | 149,000               | 21.0            | 42.2              | 38.0 |
|        | 1 hr. @ 1,500° F., FWQ+24 hrs. @ 1,200° F. | 156,200            | 151,000               | 22.0            | 40.5              | 40.0 |
|        | 2 hrs. @ 1,450° F.                         | 156,000            | 156,000               | 21.0            | 44.0              | 38.8 |
|        | 24 hrs. @ 1,200° F.                        | 155,500            | 155,500               | 22.0            | 45.2              | 38.6 |
|        | As forged                                  | 140,500            | 134,000               | 4.0             | 7.1               | 32.3 |
| K-803  | 1 hr. @ 1,700° F.                          | 131,500            | 128,500               | 4.0             | 13.9              | 32.0 |
|        | 1 hr. @ 1,400° F.                          | 134,500            | 133,700               | 3.0             | 4.1               | 29.8 |
|        | 2 hrs. @ 1,200° F.                         | 147,500            | 143,000               | 5.0             | 6.3               | 32.0 |
|        | 24 hrs. @ 1,200° F.                        | 144,300            | 144,300               | 4.7             | 34.0              |      |

It is quite evident from the inspection of Table II that the addition of the two beta stabilizers within the limits given produces an alloy of superior characteristics. For example, the tensile strength of alloy K-1025 is far superior to that of binary alloy K-803. The elongation and especially the reduction of area test proves the superiority of alloy K-1025 over and above K-803. This is most apparent when comparing the two alloys having the same heat treatment, namely, one hour at 1700° F. and 24 hours at 1200° F.

However, the above mentioned properties of these alloys are room temperature properties. It is well-known that the mechanical properties of an alloy differ at elevated temperatures from the mechanical properties measured at room temperature. In any true engineering application involving use at elevated temperatures, the me-

chanical properties of the alloy at elevated temperatures, especially creep-rupture strengths, is the usual governing criteria when selecting the proper metal to be utilized. Reference may be had to the results recorded in Table III for the outstanding creep-rupture properties of alloy K-1025 as measured at the elevated temperatures indicated.

Table III

| Heat Treatment                              | Stress<br>(p. s. i.) | Test<br>Temp.,<br>° F. | Failure<br>Time<br>(hrs.)                | El.,<br>percent | R. A.,<br>percent | Second-<br>ary Creep<br>Rate<br>(percent/<br>hr.) |
|---------------------------------------------|----------------------|------------------------|------------------------------------------|-----------------|-------------------|---------------------------------------------------|
| 15 $\frac{1}{2}$ hr. @ 1,700° F.<br>Do----- | 85,000<br>66,000     | 700<br>800             | *580 $\frac{1}{2}$<br>*547 $\frac{1}{2}$ | nil<br>nil      | nil<br>nil        | .00045<br>.00045                                  |
|                                             |                      |                        |                                          |                 |                   |                                                   |

\*Discontinued—did not rupture.

From the results recorded in Table III, it may be observed that the alloys of this invention exhibit excellent creep-rupture properties at elevated temperatures. There is very little elongation and the percent creep per hour in the test indicates excellent creep-rupture strength. It is noteworthy to point out that the alloys of this invention did not fail during the more than 500 hours at the elevated test temperatures indicated. It is also significant to observe that while these alloys have been heated to a temperature of 1700° F. and thereafter subjected to elevated temperature under stress for a prolonged period

20  
25

of time, the alloys of this invention possess excellent creep-rupture strength.

I claim:

1. An alloy consisting of, from about 6.5% to about 10% aluminum, from about 0.75% to 1.25% manganese, from about 0.75% to 1.25% chromium, and the balance titanium with incidental impurities.

2. An alloy consisting of, from about 6.5% to about 8% aluminum, from about 1% to about 1.15% manganese, from about 1% to about 1.15% chromium, and the balance titanium with incidental impurities.

3. An alloy consisting of, about 7% aluminum, about 1% manganese, about 1.15% chromium, and the balance titanium with incidental impurities.

No references cited.